

# UNITED STATES PATENT OFFICE.

JAMES E. LAPPEN, OF WINONA, MINNESOTA.

## ART OF MAKING CEMENT-FIBER BOARD.

1,297,480.

No Drawing.

Specification of Letters Patent. Patented Mar. 18, 1919.

Application filed August 5, 1916. Serial No. 113,236.

*To all whom it may concern:*

Be it known that I, JAMES E. LAPPEN, a citizen of the United States, residing at Winona, in the county of Winona and State 5 of Minnesota, have invented certain new and useful Improvements in the Art of Making Cement-Fiber Board, of which the following is a specification.

This invention relates to the art of making 10 fireproof and waterproof boards from cement and fibrous material such as asbestos and mineral wool. Such boards have many of the characteristics of stone in that they are hard and have a great resisting power 15 against atmospheric changes, pressure, and mechanical blows, and are waterproof and fireproof, while they also have other characteristics common to wooden boards, such as a certain fibrous tenacity which prevents 20 them from being easily chipped and cracked, and which makes it possible to trim or shape them by means of a saw, and to secure them to a supporting structure by simply driving 25 nails through them. Owing to the nonbrittle character of the board due to its fibrous 30 constituents such nailing can be done without cracking or chipping the board. Like wooden boards also, these cement fiber boards have a certain amount of resilience 35 which makes it possible to bend them within certain limits. All of these characteristics 40 make them especially desirable for use in place of ordinary wooden shingles.

Boards or plates of this general character 45 have heretofore been made by mixing the fibrous material, such as asbestos, with hydraulic cement in the presence of a great bulk of water, and then by building this material up layer by layer into laminated 50 plates of the desired thickness in the manner of making cardboard upon an ordinary cardboard machine, or so called "wet machine." In this way the finished product does not have a homogeneous character but 55 is in layers which can be easily detected by examining the physical structure of the product, and even the layers themselves are not homogeneous because the cement, being heavier, settles at the bottom of each layer.

Furthermore, by the use of this process the cement, being heavier, naturally settles in 60 the watery mixture, so that it comes next to the traveling apron, and will fill up the fibrous surface or pores thereof, thus clogging 65 the apron so that the water which is squeezed out from the mixture cannot get

through the apron but will run off the sides thereof and carry with it part of the material.

It is the object of the present invention, 60 among other things, to construct these fiber-cement boards in such manner that the cement does not initially come in contact with the apron at all, thereby avoiding the clogging 65 of the apron and the consequent necessity of frequently cleaning the same to remove the accumulation of cement, as well as to make the board in such way that the cement and fiber shall be intimately mixed 70 through the thickness of the board so that the product, instead of being in non-homogeneous 75 layers, will be homogeneous throughout its thickness with the cement evenly distributed among and about the fibers, without using any greater pressure 80 than such as is naturally incident to the building up of the board in the manner of the usual card-board process.

With these objects in view my process 85 consists, generally speaking, in first disintegrating the fibrous ingredients, such as asbestos and mineral wool, in water until the fibers are well separated and dispersed 90 through the water, and then, after partially draining the fibers and collecting them into a thin film, carrying the wet fibrous film under and past a source of dry cement powder and sprinkling the powdered cement 95 evenly over the surface of the film as it is carried along, and lastly building up the thin layers or films of wet fibrous material thus sprinkled with dry cement into boards or plates of the required thickness, and exerting upon them as they are being built up sufficient pressure to force the cement 100 into and through the wet fibrous mass, thereby impregnating the entire mass with cement and making it homogeneous in character.

In carrying out the process I first disintegrate the desired quantity of fibrous material in water so as to separate the fibers and put them into the vat of the well-known "wet machine" used generally for making card-board, using preferably a mixture of 105 asbestos fibers and fibers of mineral wool, and taking these fibers in the proportion of 20 lbs. of asbestos to 380 lbs. of mineral wool.

The fibers are then drawn out from the water and collected into a thin film, upon 110 the outside of the usual gauze covered revolving cylinder used in wet machines of this

character, through the application of suction to the interior of the cylinder in a manner well known in the art. At the top of its revolution the screened cylinder comes 5 in contact with a felt belting which is pressed into contact with the gauze surface of the cylinder by means of a couch roll, whereby the wet fibrous film adheres to the belt which peels it off from the gauze cylinder and carries it to and between a pair of 10 rolls, the upper of which is commonly known as the accumulator roll. During the passage of the fibrous material from the couch roll to the accumulator roll dry powdered cement is sprinkled and evenly distributed over 15 the film or stratum of wetted fiber, so as to cover the surface of the wetted material with dry powdered cement. When the cement-covered fibrous material reaches the accumulator roll it is peeled off from the belt by its greater adhesion to the accumulator roll, against which it is pressed by means of the co-acting roll on the under side of the accumulator roll. In the continued revolution 20 of the accumulator roll one layer of this cement-powdered fibrous material after another is peeled off the belt and wrapped about the accumulator roll until the accumulated layers reach the desired thickness, 25 whereupon the sheet so formed is cut from the roll in a manner well known in the art.

As the layers pass between the press rolls, meaning thereby the accumulator roll and its coacting pressure roll, this dry cement is 30 driven through the wet mass of fiber so as to come into intimate association with the fibers throughout the entire thickness of the accumulated sheet, so that the sheet will become a uniform homogeneous mass without 35 any layers that can be detected by examining the physical structure of the sheet.

It will therefore be seen that by the use of this process I avoid the difficulty which is inherent in a process where the cement and 40 fibrous material are mixed together in water before being fed to the apron or belt, of having the cement collect upon the surface of the belt and fill up the fibers or pores thereof so that the water squeezed out from 45 the mass cannot pass through the apron but washes the material out at the side; and the cement-fiber boards produced by the present process are much stronger than boards made by mixing the cement and fibers in water 50 before passing the material through the cardboard machine, because the fibers are more uniformly and thoroughly intermingled with the cement when the cement is added subsequently in dry form than they would 55

be if the cement and fibers were mixed initially with water, for this allows the cement to settle and separate out from the fibers.

The proportions of the ingredients used can be varied within certain limits but I have secured the best results by using 400 60 pounds of fibrous material to 600 pounds of cement, and I prefer to use about 20 pounds of asbestos to 380 pounds of mineral wool.

I claim:

1. The herein described process of producing cement-fiber board which consists in first disintegrating mineral fibrous material in water, then separating the disintegrated fibers out from the water and collecting them into a thin wet film, then sprinkling the surface of the film with dry cement powder, and then wrapping the film upon itself under pressure until a sheet of the desired thickness is formed.

2. The herein described process of producing cement-fiber board which consists in first disintegrating mineral fibrous material in water, then separating the disintegrated fibers out from the water and collecting them into a thin wet film, then carrying the film 75 continuously under a source of dry cement powder and sprinkling the surface of the traveling film with said powder and then wrapping the film upon itself layer upon layer and at the same time subjecting it to 80 pressure until a sheet of the desired thickness is formed.

3. The herein described process of producing cement-fiber board which consists in disintegrating a major amount of mineral wool 95 and a minor amount of asbestos in water then separating the disintegrated fibers out from the water and collecting them into a thin wet film, then sprinkling the surface of the film with dry cement powder, and then 100 wrapping the film upon itself under pressure until a sheet of the desired thickness is formed.

4. A product of the herein described process, made by first disintegrating mineral 105 fibrous material in water, then causing the wet disintegrated fibers to be spread out in a thin film, then sprinkling the film with dry cement powder, and finally wrapping the film upon itself, layer upon layer, under 110 pressure, substantially as described.

In testimony whereof I affix my signature in presence of two witnesses.

JAMES E. LAPPEN.

Witnesses:

ARTHUR P. LOTHROP,  
BEATRICE BROWN.